

Sept. 10, 1935.

J. M. JOHNSTON

2,014,356

STOCKING

Filed March 1, 1933

FIG. I.



FIG. II.



FIG. III.



WITNESSES:

John C. Bergner  
John A. Weidler

INVENTOR:

John M. Johnston  
BY Fralley & Taub  
ATTORNEYS.

## UNITED STATES PATENT OFFICE

2,014,356

## STOCKING

John M. Johnston, Elkins Park, Pa., assignor to  
 John Blood & Co. Incorporated, Philadelphia,  
 Pa., a corporation of Pennsylvania

Application March 1, 1933, Serial No. 659,076

3 Claims. (Cl. 66—202)

This invention relates to stockings; and it has reference more particularly to long hose or ladies' stockings knit from luster yarns such as silk or rayon.

5 The aim of my invention is to make possible the production of stockings of fine gage which are wrinkle and snag-proof and therefore capable of maintaining their original shape notwithstanding rough handling in use, or in laundering; 10 which are highly resistive to pulling and hence correspondingly secure against runs; and which, moreover, are characterized by an attractive subdued or semi-gloss finish.

15 As hereinafter fully disclosed, I realize the above desideratum in practice by knitting my improved stocking from a specially prepared yarn composed of a number of ends of silk whereof the majority are hard twisted individually in the same direction, and the others are untwisted, 20 and the entire group finally incorporated into the yarn by hard twisting in the direction opposite to that of the individually twisted ends.

25 Fig. I shows a lady's stocking such as may be produced as a snag and wrinkle-proof structure in accordance with my invention.

Fig. II is an enlarged diagrammatic view of a portion of the stocking fabric within the square indicated in dot and dash lines at A in Fig. I; and

30 Fig. III is an enlarged fragmentary perspective view showing the construction of the hard twist yarn from which my improved stocking is knit.

35 The stocking delineated in Fig. I is of the usual full fashioned variety capable of being produced on straight knitting machines of the "Cotton" type, it having, as usual, a welt top 10, a shaped leg 11, and a reinforced foot 12.

40 In accordance with my invention I produce a stocking of this kind from hard twist yarn 13 made after the manner illustrated in Fig. III, from three ends 14, 15 and 16 of raw silk or rayon, each such end being composed in the present instance of eight separate filaments. The ends 14, 15 I prepare initially by hard twisting them individually both in the same direction, fifty turns to the inch. With the ends 14, 15 so prepared, I associate the end 16, which, it will be noted, is without twist, and hard twist the three together sixty-five turns to the inch in the direction opposite to that of the individual ends 14, 15 aforesaid to form the yarn 13. In the present instance, the ends 14 and 15 are shown as being individually twisted to the left, and combined with the end 16 by twisting of the three to the right.

45 Incident to the knitting, the carriers of the knitting machine serve the yarn to the needles first in one direction and then in the other,—the yarn, by reason of its hard twist, relative stiffness and stability (due to the reverse twisting), lending itself to the formation, in successive courses 17 of the fabric (Fig. II), of uniformly-rounded evenly-spaced loops 18.

50 Accordingly, there results from the foregoing procedure, a stocking embodying my invention, 10 which, although very delicate in texture and appearance, is strong and durable, which is snag and wrinkle-proof and therefore capable of maintaining its original shape notwithstanding rough handling in use or in laundering; which is 15 highly resistive to pulling; and which, moreover, is characterized by a semi-gloss which adds materially to its attractiveness.

55 While I have given specific figures as to the number of twists in two of the ends incorporated 20 in the yarn and also as to the final twist of the three component ends, I do not wish to be considered as limited to these numbers since the advantages described of my new stocking may be attained by varying the initial twist of the two 25 individual ends from forty-five to fifty-five turns, and likewise varying the combining twist of the three from sixty to seventy turns per inch. It is also to be understood that my invention is not necessarily restricted to a full fashioned stocking, nor to a stocking knit with three ply yarn 30 since in the composition of the yarn the number of component ends may be varied provided that the twisting of the majority of such ends and the final twist is such as to predetermine the desired 35 results in the finished product.

Having thus described my invention, I claim:

1. As a new article of manufacture, a wrinkle and snag-proof stocking knit from yarn composed 40 of a number of ends of textile fibers such as silk, each said end including a predetermined number of filaments and the majority of which ends are twisted individually forty-five to fifty-five turns per inch in the same direction and the others untwisted, and the whole group twisted together sixty to seventy turns to the inch in a direction opposite to that of the individually twisted ends.

2. As a new article of manufacture, a wrinkle and snag-proof stocking knit from yarn composed 50 of three ends of textile fibers such as silk, each said end including a like number of filaments and two of which ends are individually twisted forty-five to fifty-five turns per inch and the third untwisted, and the three ends twisted 55

together sixty to seventy turns per inch in a direction opposite to that of the two individually twisted ends.

3. As a new article of manufacture, a wrinkle and snag-proof stocking knit from yarn composed of a definite number of ends of textile fibers such as silk, each said end including an equal

number of filaments and the majority of which ends are individually twisted fifty turns to the inch in one direction and the third untwisted, and the whole group of such ends twisted together sixty-five turns to the inch in a direction opposite to that of the individually twisted ends.

JOHN M. JOHNSTON.